

June 8, 1943.

R. BRODERSEN ET AL

2,321,279

PROCESS FOR THE MANUFACTURE OF ANTIHALATION LAYERS

Filed July 13, 1940



ANTI-HALATION LAYER CONSISTING  
OF A DYE STUFF CONTAINING AT LEAST  
ONE CARBOXY GROUP, SAID DYE STUFF  
BEING AN AROMATIC AZO COMPOUND  
OR THE CONDENSATION PRODUCT OF A  
QUINONE WITH A PHENYLENE DIAMINE

*Inventor:*

RICHARD BRODERSEN-GUSTAV WILMANNS

*by Henry W. Coughlin  
Attorney*

Patented June 8, 1943

2,321,279

# UNITED STATES PATENT OFFICE

2,321,279

## PROCESS FOR THE MANUFACTURE OF ANTI-HALATION LAYERS

Richard Brodersen, Dessau, and Gustav Willmanns, Wolfen, Germany, assignors to General Aniline & Film Corporation, New York, N. Y., a corporation of Delaware

Application July 13, 1940, Serial No. 345,368  
In Germany August 23, 1939

### 3 Claims.

This invention relates to the manufacture of antihalation layers.

In most cases it has been necessary to apply antihalation layers to photographic materials. By using a binding agent they are mostly applied to the rear of the support for the photographic emulsion in such a way, that they can be readily decolorized and removed therefrom. This procedure is connected with certain disadvantages: The thickness of the film is increased, the developer cannot completely be used up for processing, also the emulsion layer may be color-tinged and the like. Besides meeting the optical requirements, the antihalation layer must be as thin as possible, mechanically strong and also water-repellent, but on the other hand must be readily soluble in the developing baths with dyeing the developer or reducing its developing power. To a certain extent the latter happens for instance with the soluble layers described in U. S. Patent 2,161,788, as they reduce the alkali contents of the developer, in order to become soluble themselves.

The afore-mentioned requirements are fulfilled by layers consisting of dyestuff only which combine good adhering and film-forming capacity with insolubility in water and excellent solubility in the developer.

This invention has as an object the preparation of new and useful antihalation layers which are free from the above mentioned disadvantages.

A further object of the present invention is the preparation of antihalation layers possessing good film-forming capacity and being readily soluble in the developer.

These and other objects will become apparent from the following description.

As a general rule it has been found, that dyestuffs containing carboxyl groups are the ideal representatives of this group. Dyestuffs without groupings effecting solubility in the developer ( $\text{COOH}, \text{SO}_3\text{H}$ ) are not suitable, as they are very hard to remove. The comparison of quite a number of normal dyestuffs containing sulfo groups with the corresponding carboxyl dyestuffs shows furthermore the general importance of the latter grouping for the aforesaid antihalation purposes: The layers from sulfo dyestuffs, in so far as they can be prepared as a continuous layer, are always destroyed under a soft mechanical stress, especially if they are touched by moist hands. A support for the photographic emulsion, dyed by a carboxyl dyestuff, can be removed from the dyestuff only by rough mechanical means. The dyestuffs which naturally must show suitable solubility, form, if properly applied, no crystals, but an extremely fine film, the latter being firmly connected with the support for the photographic emulsion. When such photographic material is brought into the developer, the layer dissolves

### (Cl. 95—8)

spontaneously on account of the carboxyl grouping without leaving traces of the dyestuff on the support.

Which dyestuff groupings are to be used depends on the special purpose which is to be attained. If necessary, also two or more dyestuffs may be combined in one layer.

The literature reveals that two or more examples of the use of dyestuffs containing carboxyl groups are already known. It relates only, however, to the special application of a dyestuff without recognizing the general validity of the principles described.

The following are given as examples of the afore-mentioned rule:

#### (A) A comparison of the layers from

- (a) Malachite green
- (b) Chrome green
- (c) Helvetica green

20 shows that

- (a) Does not dissolve in the developer
- (b) Yields a continuous layer, is water resistant, and dissolves spontaneously in the developer
- (c) Yields a water soluble, vulnerable layer which can be rubbed off easily.

#### (B) A comparison of the three yellow-red dyestuffs



35 shows that their properties correspond to those listed in Example A.

#### (C) Layers from



60

(b)



(c)



also have the properties of (a), (b) and (c) respectively as in Example A.

(D) A comparison of



demonstrates that the properties of these dyestuffs correspond exactly to those of the above mentioned rule.

Example I

10 grams chrome green are dissolved in 500 cc. alcohol and 500 cc. propanol

and applied to a support from acetyl cellulose. 60 The layer, which is mechanically resistant and insoluble in water, dissolves readily even in a borax developer.

Example II

10 grams of the dyestuff



are dissolved in 1000 cc. alcohol and applied to glass-plates in a known manner. The violet antihalation layer thus obtained adheres firmly and does not dissolve under the influence of 5 humidity.

Example III

10 grams chrome green and 5 grams dyestuff:

10



15

are dissolved in 500 cc. alcohol and 500 cc. propanol

20 and then applied to an acetyl cellulose film. The layer thus obtained, even when wet and in contact with a photographic emulsion does not adhere to it.

Example IV

25 12 grams of a dyestuff of the following constitution



30

are dissolved in 1 liter alcohol. This solution is applied to glass-plates, which may be used for the production of panchromatic photo plates.

35 What we claim is:

1. A photographic material comprising a support, at least one light-sensitive emulsion layer and an antihalation layer consisting only of a thin film of at least one dyestuff containing in 40 its molecule at least one carboxyl group and selected from the group of dyestuffs consisting of aromatic azo compounds and condensation products of a quinone with a phenylene diamine.

2. A photographic material comprising a support, at least one light-sensitive emulsion layer, 45 and an antihalation layer consisting only of a thin film of a dyestuff having the following formula

50



55

3. A photographic material comprising a support, at least one light-sensitive emulsion layer, and an antihalation layer consisting only of a thin film of a dyestuff having the following formula



RICHARD BRODERSEN.  
GUSTAV WILMANNS.